

May 18, 1965

A. F. PRUST

3,184,326

COATING OF IRON AND STEEL

Filed June 10, 1960



ALVIN F. PRUST  
INVENTOR.

BY  
William H. Woodling  
HIS ATTORNEY

3,184,326

## COATING OF IRON AND STEEL

Alvin F. Prust, Warren, Ohio, assignor to Republic Steel Corporation, Cleveland, Ohio, a corporation of New Jersey

Filed June 10, 1960, Ser. No. 35,326

12 Claims. (Cl. 117—51)

This invention relates to improvements in the formation of aluminum coatings on iron and steel. More particularly, it relates to an improved process and improved pretreating composition for forming a uniform and well-adhered coating of aluminum on the iron or steel.

An aluminum coating on iron and steel provides excellent protection against corrosion. However, although numerous methods have been proposed for applying such coatings, they leave something to be desired for commercial use, either because of erratic or unsatisfactory results in the process and product, or because of the expense involved in the materials used or the method of application. Furthermore, toxic fumes from some of the materials used in certain processes have helped to make such processes even less attractive.

Some of the proposed methods utilize a molten aluminum bath in which the steel is immersed after it has been treated in molten salt fluxes. Another suggested method calls for keeping the surface of the steel wet with water until it is to be immersed in molten aluminum.

Another proposed method involves a pretreatment with an aqueous solution or suspension of sodium fluosilicate, potassium chloride, sodium chloride, and sodium fluoride, or cryolite. A more recent suggestion recommends pretreating with an aqueous solution of zinc chloride together with various other chlorides.

In spite of the variety of salts and the variety of combinations of such salts recommended as pretreating fluxes and the various methods of pretreatment recommended, the proposed methods are not particularly suited to commercial use either because of expense, complicated procedures, or inefficient results.

It has now been found that an aluminum coating can be applied to iron and steel very efficiently and inexpensively by applying to a freshly cleaned iron or steel surface, preferably at a temperature of about 170—190° F., an aqueous solution containing approximately 1.3—6.0 ounces of an alkali metal fluoride, such as sodium fluoride, and approximately 1.3—6.0 ounces of a stannous salt, such as stannous chloride, stannous fluoride, stannous sulfate, etc. per gallon of solution, together with sufficient acid to keep the pH between 3.5 and 4.0 (0.6 to 2.8 ounces of 22° Baumé hydrochloric acid per gallon of solution), removing excess solution, drying the aqueous film on the metal, and then introducing the metal into molten aluminum. The process is adaptable to batch, semi-continuous, or continuous operation.

While it is not intended that the invention be restricted to such a theory, it is believed that the stannous salt and the alkali metal fluoride react to form a complex fluoride, such as  $\text{Na}_2\text{SnF}_4$ . This complex fluoride is in a form which is resistant to hydrolysis in the presence of water and forms a chemical-barrier layer on the surface of the metal. This thin, chemical-barrier layer dispenses with the need for a heavy deposition of the various fluxes previously used which generally resulted in porosity problems due to the failure of such fluxes to adhere and uniformly coat the metal base. While the corresponding alkali metal stannous fluoride is similarly effective when the lithium or potassium fluoride is used, it is preferred to use sodium fluoride which is more easily available and more economical. Although other acids, such as sulfuric acid and phosphoric acid, also can be used for

this purpose, it is generally preferred to use hydrochloric acid to maintain the desired pH.

Before the iron or steel surface is treated, it must be cleaned entirely of foreign materials, such as oxide coatings, greases, etc. Various pickling procedures can be used for this purpose. A preferred method of cleaning is to immerse the iron or steel for approximately 15 to 90 seconds in about 8—10% sulfuric acid at about 180—190° F. Any equivalent method of obtaining a clean surface is satisfactory.

Various types of steel can be used in the process, including various carbon steels, silicon steels, low alloy high-strength (such as those containing 1.0% copper, 1.0% nickel, 0.15—0.20 molybdenum), etc. The iron or steel can be in various shapes, and either unfabricated or fabricated articles can be used in the process. In continuous modifications of this process, the steel advantageously is in strips, ribbon, wire, or other form adapted to be stored in roll form prior to being advanced through the various processing steps. Also, fabricated articles can be run through the sequence of treating steps on a conveyor device.

Although the various proportions of the salts will operate in accordance with the range indicated above, it generally is advantageous to have approximately equal parts by weight of the stannous salt and the alkali metal fluoride. A preferred composition has 3.0 ounces of sodium fluoride and 3.0 ounces of stannous chloride per gallon of solution, with sufficient hydrochloric acid therein to give a pH of 3.5—4.0. Approximately, 1.4 ounces of 22° Baumé hydrochloric acid per gallon of solution gives the desired pH range. While higher concentrations of these salts also are operative, these concentrations are the most economical.

Various methods of applying the aqueous liquid film to the metal surface can be used. Where convenient the metal object can be immersed in the liquid and excess liquid allowed to run off the article after its removal from the bath. Sheets, ribbons, wires, or filaments of the metal can be run continuously below the surface of the aqueous bath and excess liquid allowed to run off after the metal has passed through the bath, or can be squeezed off by passing the metal between two rollers. The aqueous liquid also can be applied to the surface of the metal by flowing the liquid over the metal, or by spraying the liquid thereon.

While it is generally desirable to have both the metal and the solution approximately at a temperature in the range of about 170—190° F., it is possible also to have one or the other outside this range, providing the resultant temperature of the flux and metal during the contact time is approximately the temperature indicated. Treating bath temperatures as high as 400° F. have been found satisfactory. An immersion or contact time of 6—10 seconds generally is satisfactory to give the desired flux film.

After the metal has been in contact with the aqueous solution, it is necessary that the resulting aqueous film be dried on the surface of the metal by evaporation of the water as soon as possible and prior to having the metal pass over any roll other than the squeegee roll used to remove excess liquid. Various methods of drying the aqueous film can be used provided the film is not rubbed off the metal surface. Radiation from heated surfaces or heat lamps and currents of warm air are found particularly advantageous for this purpose.

Within ten minutes after drying, and preferably as soon as possible after drying, the resultant metal surface should be immersed in the molten aluminum. Abrasion of the metal surface should be avoided as much as possible although very minor abrasions will not disturb the dried film sufficiently to prevent aluminum coating.

The flux of this invention is not sensitive to exposure to ambient atmospheric conditions. Strip has been coated commercially satisfactory as to porosity and formability, after being exposed to air up to 20 minutes between fluxing and dipping in the aluminum bath. It has been ascertained further that strip or articles coated with this flux can be preheated before immersion in the molten aluminum metal with no deleterious effects upon the resultant coating. In this way, less heat input to the molten aluminum pot is necessary.

A thickness of film sufficient to give complete coverage without any pinholes or bare spots is desired. Such coverage is obtained by observing the conditions described herein. Since complete reaction between the molten aluminum and the dried film is desirable, a salt film of excessive thickness is not desirable. An immersion period of 5-15 seconds in the molten aluminum bath is generally satisfactory, although a shorter period of 3 or 4 seconds is sometimes desirable.

The temperature of the metal strip entering the aluminum bath is generally not over 150° F. However, this can vary according to the flux bath temperature and according to the temperature developed during the subsequent drying step.

The temperature of the aluminum bath advantageously is sufficiently above the melting temperature of the aluminum or aluminum alloy therein so as to compensate for heat loss to the metal passing through the bath as well as to normal losses to the surroundings. However, for economy of heat and of time in cooling the coated product, it is generally not desirable to maintain a molten aluminum temperature greatly in excess of that required to keep the aluminum in a molten condition.

Generally a temperature in the range of about 1275° F. to 1330° F., preferably about 1280°-1290° F. is economical and satisfactory.

When the aluminum bath is maintained at a temperature substantially below 1280° F., the metal strip cools the bath at the area where it enters the bath so that a semi-solid mushy deposit builds up in this area. At an aluminum bath temperature of 1330° F., the resultant product has an oxidized surface, indicated by a gold cast. While neither of these effects is completely objectionable, it is desirable to stay at least five degrees within the extremes of this temperature range, preferably about 1280°-1290° F.

Where it is desired to coat the iron or steel with an aluminum alloy, such as for example, aluminum silicon, the corresponding aluminum alloy molten bath will be used and the temperature modified accordingly.

After the metal is coated it is cooled by exposure to the atmosphere. It is generally desirable to allow at least 25 feet before the sheet comes in contact with a guide roll. If desired, forced air cooling can be effected.

When the product is to be rolled or coiled, the coated product can have a temperature as high as about 400° F. although temperatures of 120-165° F. are generally advantageously effected. This temperature is determined by the temperature of the metal at entry to the cooling chamber, the temperature of the cooling medium, and the period of cooling.

A typical pretreating and coating operation with a roll of 0.060 gauge cold-rolled steel is described below in relation to the schematic flow-sheet shown in the accompanying drawing illustrating a continuous coating process according to the practice of this invention. The roll is supported in such a manner that it is free to rotate on its axis with the sheet passing through driven pinch rolls so as to move the sheet forward. The sheet then is passed over guide rolls and then into a pickling bath of such dimensions that the metal has a residence time therein of approximately 60 seconds.

The pickling bath is about 8-10% sulfuric acid, maintained at 180°-200° F. After the pickling bath, the sheet

passes through a water rinsing stage to remove residual acid. Rinse water at temperatures normally delivered from water mains (approximately 50°-110° F.) is satisfactory although rinse water temperatures as high as 180° F. can be used provided evaporation is avoided before the strip is covered or fed into the treating bath. If desired the pickling operation can be carried out separately, provided the metal is kept clean and is not stored long enough to pick up any oxide coating. The pickling and rinsing stages are not shown in the drawing.

The drawing is a diagrammatic representation or flow sheet of one mode of carrying out the process.

Then the sheet 1 coming from the aforesaid rinsing stage or from a storage roll, is passed over guide roll 2 into a treating bath 3 in container 4 of such dimensions as to give the metal approximately a 10 second residence time in the bath. The sheet is passed under a second guide roll 5. The bath contains 3.0 ounces of sodium fluoride, 3.0 ounces of stannous chloride, and 2.5 ounces of 22° Baumé hydrochloric acid per gallon of solution. The pH is checked periodically and additional acid added when necessary to maintain a pH in the range of 3.5-4.0. The bath temperature is maintained in the range of approximately 170° F. to 190° F.

After leaving the aqueous bath, the sheet is passed through rolls 6 to remove excess aqueous film, then passed between two banks of heating lamps 7 to effect drying of the film. Guide roll 8 is spaced far enough from the banks of lamps that the water is completely evaporated from the film before the sheet comes into contact with it. Stack 9 is provided in enclosure 10 for escape of the moisture laden air. If desired, forced ventilation can be provided.

Then the sheet is passed over guide roll 11 and under guide rolls 12 and 12', into a molten aluminum bath 13 maintained at a temperature of approximately 1280° F. and of such dimensions that the sheet has a residence time of approximately 5 seconds.

After emerging from the molten aluminum bath, the sheet passes upward through a distance of about 25 feet and is cooled by exposure to the atmosphere so that the temperature is reduced to approximately 120°-165° F. Then, after passing over guide roll 14, the cooled, coated product is rolled and stored on the driven storage roll 15.

The resultant product is found to have excellent adhesion of the aluminum coating to the metal base and upon fabrication into various shapes exhibits excellent adhesion of the coating to the base without any cooling or cracking of the coating. Similar continuous processing of iron and steel wire and ribbon gives similar coated products which can be bent on an extremely small radius without causing cracking or peeling of the coating. Strips coated in this manner can be cold rolled to a bright luster and can be drawn or shaped by any conventional means without flaking of the aluminum coating.

The foregoing description is merely illustrative and various modifications are obvious.

While certain features of this invention have been described in detail with respect to various embodiments thereof, it will, of course, be apparent that other modifications may be made within the spirit and scope of this invention and it is not intended to limit the invention to the exact details shown above except insofar as they are defined in the following claims.

The invention claimed is:

1. An aqueous pretreating solution for improving the adhesion of an aluminum coating to a ferrous base consisting essentially of about 1.3-6.0 ounces of alkali metal fluoride and about 1.3-6.0 ounces of a stannous salt per gallon of aqueous solution maintained at a pH in the range of about 3.5-4.0.
2. A solution of claim 1 in which said stannous salt is stannous chloride and said fluoride is sodium fluoride.
3. A solution of claim 2 in which said pH is maintained with hydrochloric acid.

4. A solution of claim 2 in which said proportions of said sodium fluoride and said stannous chloride are approximately equal.

5. A solution of claim 4 in which said pH is maintained with hydrochloric acid.

6. A process for applying an aluminum coating to a ferrous metal comprising the steps of applying a film of an aqueous solution to a ferrous metal surface, said solution consisting essentially of about 1.3-6.0 ounces of an alkali metal fluoride and about 1.3-6.0 ounces of a stannous salt per gallon of aqueous solution, said solution having a pH in the range of about 3.5-4.0, immediately thereafter evaporating the water from said solution, and then immersing said dried metal surface in a molten aluminum bath for a period sufficient to apply a coating of desired thickness.

7. A process of claim 6 in which said stannous salt is stannous chloride and said fluoride is sodium fluoride.

8. A process of claim 6 in which said pH is maintained with hydrochloric acid.

9. A process of claim 7 in which said sodium fluoride and said stannous chloride are present in said solution in approximately equal proportions by weight.

10. A process of claim 9 in which said pH is maintained with hydrochloric acid.

11. A process of claim 10 in which said aqueous film is applied at a temperature in the range of approximately 170°-190° F.

12. A process of claim 6 in which said aqueous film is applied at a temperature in the range of approximately 170°-190° F.

References Cited by the Examiner

UNITED STATES PATENTS

|           |       |                |       |           |
|-----------|-------|----------------|-------|-----------|
| 527,478   | 10/94 | Broadwell      | ----- | 117-51    |
| 2,671,737 | 3/54  | Jominy et al.  | ----- | 117-51    |
| 2,706,161 | 4/55  | Westby         | ----- | 117-52    |
| 3,027,269 | 3/62  | Teshima et al. | ----- | 117-114 X |

RICHARD D. NEVIUS, Primary Examiner.

JOSEPH B. SPENCER, Examiner.